

Sept. 20, 1932.

G. A. REINHARDT ET AL

1,878,540

ELECTROLYTIC METHOD OF CONTINUOUS SHEET MANUFACTURE AND APPARATUS THEREFOR

Filed March 22, 1929



WITNESS

*H. J. Hartmann.*

BY

*Blank & Stellard*

ATTORNEYS

INVENTORS  
Gustav A. Reinhardt,  
Richard H. Eutrich.

## UNITED STATES PATENT OFFICE

GUSTAV A. REINHARDT AND RICHARD H. EURICH, OF YOUNGSTOWN, OHIO

ELECTROLYTIC METHOD OF CONTINUOUS SHEET MANUFACTURE AND APPARATUS  
THEREFOR

Application filed March 22, 1929. Serial No. 349,070.

Our invention relates to continuous electrolytic production of relatively thin sheets of indefinite length and of any desired width, the principal object of the invention being to provide a satisfactory commercially operative method for the production of such sheets as well as apparatus suitable for the performance thereof.

While our invention lends itself to the production of both ferrous and non-ferrous sheets, it is particularly adapted for the production of the former and we will therefore refer herein more especially to its use for that purpose. Hitherto the commercial production of such sheets has involved a tedious series of rolling and like operations by means of which a billet containing suitable amount of metal is gradually and progressively reduced to a sheet of the desired size and thickness. In accordance with our invention, however, the sheet is directly and continuously formed either of the ultimate desired width and thickness or else of slightly greater thickness so that it may readily be reduced to the ultimate desired thickness by one or more passes through suitable rolls which may also serve to impart desired physical characteristics or finish, or both.

To enable those skilled in the art to comprehend and practise our invention we will now describe one manner of performing our method of electrolytically producing continuous sheets, reference being had to the accompanying drawing in which we have diagrammatically illustrated one form of apparatus suitable for the performance thereof, the single figure being a transverse vertical section through the apparatus with certain of the parts thereof shown in elevation.

In accordance with the preferred practice of our invention the formation of the sheet is effected by continuous electrolytic deposition of metal on a revolving cathode from an anode submerged in a suitable electrolyte and formed of ferrous material and then stripping the deposit from the cathode in the form of a continuous sheet of indefinite length after removing at least a large portion of the hydrogen which is included or entrained within the metal as it is progressively depos-

ited, and which if allowed to remain therein would prevent satisfactory stripping of the sheet as well as render the latter substantially unfit for immediate use or further finishing operations.

More particularly and as shown in the drawing we provide a tank or vat 1 of any suitable construction and lined or otherwise protected if necessary from the action of the electrolyte to be employed and which may desirably be a solution of ferrous chloride or other ferrous salt. This tank is of greater length than the width of the sheet to be formed and is filled with the electrolyte E to a suitable depth. Disposed within the tank in such position that it will be to a large extent submerged by the electrolyte is a cylindrical mandrel 2, desirably a cast iron roll of relatively large diameter, for example ten feet or more, though under some circumstances mandrels of lesser diameter may be satisfactorily employed; to effect a saving in weight the mandrel may be hollow but its outer surface should be smoothly finished throughout its extent. This mandrel is mounted on a horizontal shaft 3 in turn supported in suitable bearings (not shown) and arranged to be driven at a relatively low speed by suitable driving means so as to correspondingly rotate the mandrel in the direction indicated by the arrow. The bearings or journals for the shaft 3 may be supported by the end walls of the tank or in any other suitable way and through them the necessary electrical connection with the mandrel, which acts as the cathode during the electrolytic formation of the sheet, may be conveniently effected. These connections, as well as others hereinafter described, are not illustrated in the drawing since they may be effected in any of the several ways commonly practised in the electroplating art and which are well understood by those conversant therewith.

Within the tank is also disposed an anode 5; this anode is desirably curved in conformity with the surface of the mandrel and arranged to extend adjacent thereto from a point a little below that at which the mandrel enters the electrolyte to a point con-

55

60

65

70

75

80

85

90

95

100

siderably beyond its vertical diameter and as the anode is of course approximately the same length as the mandrel substantially one-half the surface of the latter is thus in juxtaposition with the anode which when the deposited metal is to be taken therefrom, as is customary in the electrolytic deposition of iron, should be formed of iron of maximum solubility under the conditions present and of low internal resistance. Thus an anode formed of that type of iron known as sponge iron may desirably be employed, but anodes formed of other ferrous materials may be used if preferred.

As in the case of the mandrel or cathode, the anode 5 is suitably connected to a source of direct current in any convenient way.

Thus as the mandrel is slowly revolved in the direction of the arrow while the current is flowing, metallic iron is progressively deposited on the surface of the mandrel as it moves past the anode so that a continuous film or layer D of progressively increasing thickness is formed on the mandrel which, after it is stripped from the mandrel as hereinafter described, constitutes the formed sheet S. This metallic iron deposit adheres quite tenaciously to the mandrel and we therefore provide means for loosening it therefrom, said means desirably comprising a roll 6 of a length approximating that of the mandrel but preferably of considerably smaller diameter. This roll is mounted on a suitably journaled shaft 7 extending parallel with the mandrel shaft 3 and so disposed that the roll 6 will bear on the layer of deposited metal preferably substantially at the top of the mandrel; suitable means (not shown) are provided for driving the shaft 7 and in turn the roll 6 preferably in the opposite direction to the mandrel and means may also desirably be arranged for regulating the pressure of the roll 6 upon the layer of metal. The speed of rotation of the roll 6 is ordinarily so adjusted that its surface speed is somewhat different from that of the layer of metal passing beneath it with the result that the latter is loosened from the mandrel and the upper surface of the sheet or layer to some extent smoothed and polished thereby. Additionally for positively freeing the sheet from the mandrel we provide a stripper 8 comprising a sharp edge at its forward end which extends beneath the roll between the mandrel and the sheet so as to raise the latter from the mandrel just after it leaves the roll; desirably the upper forward face of the stripper, which of course extends for the full length of the mandrel, is beveled rearwardly and upwardly so as to direct the sheet angularly upward away from the mandrel, from whence it is led to a reel or other suitable mechanism adapted to progressively receive it as it is discharged from the mandrel.

As deposited on the mandrel, the metal

is extremely brittle or "short" and thus not suitable for the subsequent stripping operation since the roll 6 or other means employed to loosen the metal from the mandrel would crack or break up the deposit and thus prevent the formation of a continuous sheet. This shortness or brittleness of the metal is due principally to the presence of hydrogen which is included in the metal as it is deposited electrolytically upon the mandrel and we therefore provide means for removing all or at least the major portion of this hydrogen from the deposited metal before it is subjected to the stripping operation.

While the means provided for effecting this hydrogen removal may be of any character suitable for the performance of the intended function, one form satisfactorily operative for the purpose comprises an electrode 10 desirably curved in conformity with the mandrel and disposed adjacent the surface of the latter below the point at which it leaves the electrolyte as it rotates. This secondary electrode is immersed in a portion E' of the electrolyte which is disposed in a separate cell and thus kept apart from the major portion thereof in the tank 1 in any suitable way, for example and as shown, by providing in the tank at a suitable distance below its top a horizontal longitudinally extending partition 11 whose inner edge terminates adjacent the mandrel and is provided with a flexible gasket 12 of rubber or like material whose free edge turns up against the surface of the metal deposit on the mandrel and forms a substantially liquid tight seal at this point so as to prevent any material mixing of the electrolyte E' above the partition with the major portion of the electrolyte E in the tank. The electrode 10 is so electrically connected that its potential is negative as respects the mandrel and deposit D thereon whereby as the mandrel moves past the electrode a reversal of the current flow is effected and the major portion of the hydrogen in the deposited metal as well as a small amount of the deposited metal itself is carried over to the electrode and the balance or major portion of the deposited metal on the mandrel thus freed from the gas so that it leaves the electrolyte substantially devoid thereof.

We also prefer to arrange a flash annealing mechanism above the tank in such position that a hot flame projected by this mechanism will play across the width of the surface of the deposited metal before the latter reaches the roll 6; this flash annealing mechanism, generally designated as 14 and which may be of any suitable construction, extends substantially the full length of the mandrel and performs to some extent a double function, namely, that of removing any residual hydrogen which may not have been removed by the action of the electrode 10 and of an-

nealing the deposited metal through the application of heat to thereby enhance its toughness and flexibility and thereby facilitate the stripping operation. While we prefer to employ both the electrode 10 and flash annealing mechanism as described, in some cases either one or the other may be found sufficient to remove enough hydrogen from the metal to permit it to be stripped from the mandrel.

It is also possible to effect removal of the hydrogen either in conjunction with the flash annealing mechanism or without it by impressing on the direct current utilized to effect the deposition of metallic iron on the mandrel a suitable alternating current as has heretofore sometimes been practised in the plating art and we therefore contemplate the use of this method of removing the hydrogen under conditions which might make the same desirable and include the same within the scope of our invention. Of course when this method of hydrogen removal is employed the electrode 10 and partition 11 or other means utilized to form a separate cell for its reception will ordinarily be omitted.

As it is believed the manner of practising our improved method of electrolytically forming continuous sheets by the use of an apparatus such as we have described will be readily apparent from the foregoing, extended reference thereto would be superfluous. It should be noted, however, that sufficient metal to form a sheet of the desired thickness must be deposited on the mandrel between the time when any given point thereon receives its initial deposit, which occurs when the point is adjacent the upper end of the anode 5, and the time when it passes from the depositing zone near the other end of the anode; consequently, the rotational speed of the mandrel must therefore be adjusted to effect this result under the particular conditions as to current strength and the like which may be present. Additionally, depending on how much of the deposited metal is removed through the operation of the electrode 10 if employed, some allowance may also have to be made for a corresponding reduction in thickness of the deposit resulting therefrom and therefore, where the amount of metal so removed is appreciable, it is requisite that the thickness of the deposit before this removal is effected be slightly greater than the desired ultimate thickness of the sheet.

Although we have herein more particularly referred to the use of our invention in the production of a continuous ferrous sheet when using an anode soluble in the electrolyte to supply the deposited metal, it is to be understood that, if desired, an anode insoluble in the electrolyte may be used instead and the metal derived from the electrolyte itself, and further, that by the use of a suitable

electrolyte and an anode of proper material, our invention may be employed with equal facility for the production of non-ferrous sheets. Thus, for example, a solution of zinc salt may be used as the electrolyte in conjunction with a soluble zinc anode instead of a ferrous anode to produce a continuous zinc sheet, or a suitable solution of zinc salt in conjunction with a lead or other anode insoluble therein may also be employed for a similar purpose, the deposited metal in that case being abstracted from the solution instead of from the anode.

Moreover, while we have herein described one manner of performing the invention together with apparatus suitable therefor, we do not thereby desire or intend to specifically confine or limit ourselves thereto as modifications may be made in the method itself and changes and variations in the constructional details of the apparatus may also be effected if desired without departing from the spirit and scope of the invention as defined in the appended claims.

Having thus described our invention, we claim and desire to protect by Letters Patent of the United States:

1. The method of forming a metallic sheet of indefinite length which comprises the steps of forming an electrolytic metallic deposit progressively on the face of a mandrel rotating in an electrolyte until the deposit attains a predetermined thickness, thereafter removing included hydrogen from the deposited metal and then immediately removing the latter from the electrolyte and stripping it from the face of the mandrel as a continuous sheet.

2. The method of forming a ferrous sheet of indefinite length which comprises the steps of rotating a cylindrical mandrel in an electrolytic bath, forming an electrolytic deposit of ferrous metal on the face of the mandrel progressively as it moves through the electrolyte until the deposit attains a predetermined thickness, removing from the deposit, included hydrogen, immediately thereafter removing the deposit from the electrolyte then loosening the deposit from the mandrel by application of pressure and finally stripping the deposit from the mandrel as a continuous sheet.

3. The method of forming a ferrous sheet of indefinite length which comprises the steps of rotating a cylindrical mandrel of relatively large diameter through an electrolytic bath containing an anode, forming an electrolytic deposit of progressively increasing thickness on the face of the mandrel as it moves past the anode, effecting removal of included hydrogen from the deposit electrolytically after obtaining its desired thickness, removing the dehydrogenized deposit from the electrolyte, then loosening the deposit from the mandrel by application of roll

pressure and finally stripping the deposit from the mandrel as a continuous sheet.

4. The method of forming a ferrous sheet of indefinite length which comprises the 5 steps of rotating a cylindrical mandrel adjacent an anode and an electrode respectively disposed in separate cells, forming an electrolytic deposit of ferrous metal on the surface of the mandrel while it is passing said 10 anode, passing an electric current between the mandrel and the electrode to thereby remove included hydrogen from the deposit while it is passing the electrode and immediately preceding its leaving the electrolyte, 15 then subjecting the deposit to roll pressure to loosen it from the mandrel and finally stripping the deposit therefrom as a continuous sheet.

5. In apparatus for electrolytic formation 20 of continuous metallic sheets, an electrolytic cell, a cylindrical mandrel of relatively large diameter adapted for partial immersion in and rotation through the electrolyte in the cell, an anode disposed in the cell adjacent 25 the face of the mandrel, electric connections between the anode, mandrel and a source of direct current, means for removing included hydrogen from metal deposited on the face of the mandrel comprising an electrode disposed 30 adjacent the mandrel and beneath the surface of the electrolyte and heating means disposed adjacent the mandrel above the surface of the electrolyte, means for loosening the deposited metal from the mandrel after 35 said hydrogen removal, and means for thereafter stripping the deposited metal from the mandrel as a continuous sheet.

6. In apparatus for electrolytic formation of continuous sheets, a rotatable cylindrical mandrel, a vat partially enclosing said mandrel and forming in combination therewith separate cells respectively adapted to contain an electrolyte, an anode disposed in that cell first traversed by the surface of the mandrel as it rotates, an electrode disposed in the other cell, means disposed between the cells operative to prevent passage of the electrolyte therebetween, a roll disposed above the mandrel and arranged to bear vertically 50 downward thereon to loosen the layer of deposited metal as it moves under the roll, and stripping means in the rear of the roll operative to strip the loosened layer of metal from the mandrel as a continuous sheet.

55 7. In apparatus for electrolytic formation of continuous sheets, a rotatable cylindrical mandrel, a vat partially enclosing said mandrel and forming in combination therewith separate cells respectively adapted to contain an electrolyte, an anode disposed in that cell first traversed by the surface of the mandrel as it rotates and having a positive potential with respect to the mandrel, an electrode disposed in the other cell and connected 60 to the mandrel through a source of current

whereby current is caused to flow through the electrolyte between said electrode and the mandrel, a roll disposed above the mandrel and arranged to bear vertically downward thereon to loosen the layer of deposited metal as it moves under the roll, and stripping means in the rear of the roll operative to strip the loosened layer of metal from the mandrel as a continuous sheet.

8. In apparatus for electrolytic formation 75 of continuous sheets, a cylindrical mandrel arranged to rotate through separate bodies of electrolyte, an anode immersed in the first of said bodies encountered by the mandrel as it rotates and having a given potential with respect to the mandrel, an electrode immersed in the other body and having an opposite potential with respect to the mandrel, a roll disposed above the mandrel and operative to bear on the surface of the layer of metal deposited on the mandrel during its passage through the first body of electrolyte and after its emergence from the second body thereof to thereby loosen the metal from the mandrel, means operative to anneal the metal by application of heat before it reaches the roll, and means operative to strip the layer of metal from the mandrel as a continuous sheet after it has been acted upon by the roll, said electrode being operative to abstract included hydrogen from the deposited metal during its passage through the second body of electrolyte.

In witness whereof, we have hereunto set 80 our hands this 19th day of March, 1929.

GUSTAV A. REINHARDT.  
RICHARD H. EURICH.

100

105

110

115

120

125

130